

## UNITED STATES PATENT OFFICE

2,207,879

METHOD OF MAKING SEMIPYROPHORIC  
IRON AND THE PRODUCT OBTAINED  
THEREBY

Alfred Schmid, Berlin-Dahlem, Germany, assignor to Oswald F. Wyss, Zurich, Switzerland

No Drawing. Original application August 27, 1932, Serial No. 630,702. Divided and this application August 11, 1937, Serial No. 158,593. In Germany August 28, 1931

## 2 Claims. (CL 75—33)

This application is a divisional of my copending U. S. application, Serial No. 630,702, filed August 27, 1932 now U. S. Patent 2,096,009, dated October 19, 1937.

5 This invention relates to a method of producing semipyrophoric iron and the product obtained thereby, and has for its main object to provide a safety ignition mixture, the combustion of which takes place without flame and without 10 the production of poisonous or bad smelling gases or of both.

The known ignition mixtures used for starting combustion processes generally consist of the following constituents:

15 (a) Easily decomposable substances yielding oxygen by decomposition, such as chlorates, nitrates, chromates, peroxides, and the like.

(b) Substances easily inflammable at low temperatures such as phosphorus, sulfur, carbon or 20 compounds of the same.

(c) Additions of hard and chemically inert substances increasing friction, such as quartz, clay, pumice stone and the like.

(d) Binding agents such as glue, starch, gum 25 arabic and the like.

(e) Substances preventing an explosive combustion such as zinc oxide, iron oxide and the like.

30 Due to the presence of the substances mentioned under b, all known ignition mixtures are combusted with flames and evolution of poisonous or evil smelling gases or of both. Their use is therefore impossible in all those cases, where open flames or the evolution of gases are dangerous or noxious.

35 The present invention provides for a safety ignition mixture which may easily be ignited on the usual friction surfaces for safety matches and are combusted without flame and without evolution of noxious or evil smelling gases. Self-ignition of the new ignition mixtures is impossible. The new ignition mixtures are especially suitable as igniting-heads for cigars, cigarettes and matches, which are safely and efficiently 40 lighted by more friction on one of the usual friction surfaces for matches, which surfaces are preferably arranged on or in the packages for the cigars, cigarettes or matches.

45 According to the invention the phosphorus, sulfur or the like present in the known ignition mixtures is replaced by metals with a sufficiently low ignition temperature such as magnesium, aluminium, zinc, iron, cobalt and the like, which on combustion do not furnish volatile combustion products but solid oxides in form of a powder.

The main feature of the new ignition mixtures is the absence of phosphorus, sulfur, carbon or their compounds, the inflammability of the mixture being solely due to the combination of oxygen yielding substances with easily ignitable 5 metals.

For many purposes ordinary metals would yield ignition mixtures, the ignition of which would be too difficult for the purpose in question. The invention provides for means to bring these 10 metals into a form, in which their rapid oxidation or combustion is facilitated.

15 It is known, that certain metals such as iron or cobalt may be obtained in the pyrophoric form by reducing at relatively low temperatures suitable compounds of these metals with streaming hydrogen. These pyrophoric metals are, however, ignited and combusted by contact with oxygen or air at room temperature. This pyrophoric form of metals is not suitable for the purpose of 20 the invention and the invention therefore has for its further object, to provide for a method, which enables the manufacture of metals in such a form, that they may be ignited with air at temperatures above atmospheric temperature, 25 preferably above 50° C., but below 300° C. I have named this form of metals "semipyrophoric," which is an intermediate form between pyrophoric and normal form. This method for making semipyrophoric metals consists in a reduction 30 of metal compounds suitable for the manufacture of pyrophoric metals under such modified reducing conditions that neither the pyrophoric nor the normal form is obtained or in treatment of pyrophoric metals which makes them more 35 difficultly ignitable. The reduction of the metal compounds may be carried out by thermal decomposition in presence of inert gases or by treatment with hydrogen at raised temperatures.

40 A metal is "semipyrophoric" when, on the one hand, it is not self-ignitable by mere contact with air and, on the other hand, is not so difficultly ignitable as in the normal state but can be brought into a state of ignition by friction on a friction surface. Or, in other words, a metal is 45 "semipyrophoric" when its ignition temperature

(1) Is not so low that it ignites by contact with air at room temperature;

(2) Is not so high that it does not ignite by friction on a specially prepared friction surface;

(3) But is of such a nature that mere friction on a specially prepared friction surface is sufficient for igniting the metal.

Temperature and duration of these treatments must be kept within limits, outside of which 55

pyrophoric or normal metals are obtained. Starting materials for the method according to the invention are inorganic or organic metal compounds such as oxides, nitrates, carbonates, sulfates, oxalates, tartrates or the like.

5 Pyrophoric metals may be converted into semipyrophoric metals by a shorter or longer heat treatment in the presence of inert gases, such as nitrogen, hydrogen and the like.

10 For the manufacture of semipyrophoric metals the duration of the treatment is a function of the temperature. Moreover temperature and duration of the treatment are different for different metals, gases and pressures employed. It 15 is therefore not possible to give general data for temperature and duration of the treatment, but the following examples may lead the expert in finding the conditions for making semipyrophoric metals other than iron or semipyrophoric iron 20 from other starting materials or by a modified method.

*Example I*

10 gr. of ferrous oxalate are heated to about 25 400° C. in streaming hydrogen, which has been dried by passing it through concentrated sulfuric acid before entering the reaction zone and which passes this zone at a moderate rate corresponding to about two gas bubbles leaving the sulfuric acid per second.

30 When the amount of gases leaving the reaction zone decreases, which is the case after about one hour, the reaction is finished. The heating is stopped and a rapid cooling is effected by passing hydrogen through the reaction zone. When room 35 temperature has been reached a black powder is obtained not ignitable by contact with air, at room temperature, but ignitable, when contacting it with air at about 180° C.

*Example II*

40 28 parts of the semipyrophoric iron produced in the manner described are mixed with 25 parts of potassium chlorate, 1 part of pyrolusite and 18 parts of powdered burnt clay. The mixture is

powdered and mixed while stirring with 80 parts of a 4% solution of collodion in volatile organic solvents, some ether and alcohol being added to the pappy mixture if necessary. The mixture is placed on the top of a cigar or cigarette in any 5 convenient manner, thus obtaining a firmly adhering ignition head on the article after evaporation of the volatile solvent in the air.

The igniting mixture described above may contain other substances, such as fillers and the like, or may be combined with other pyrotechnic mixtures. It may be arranged on any inflammable carrier and thus serve to light any combustible substance.

15 The solution of collodion employed as binding agent in the above example may be replaced by solution of other binders, such as acetyl cellulose and the like, in volatile organic solvents, such as alcohol, ether, acetone, amyl acetate and the like. Also aqueous solutions of glue, starch, gum arabic and the like may be employed, although binders containing volatile organic solvents are preferred, as the solidification of the ignition mixtures on their carriers is accelerated, when the binder contains volatile liquids as solvent. The amount of binder used is kept as low as possible and preferably such binders are employed, which are easily and completely combusted without the evolution of noxious or bad smelling gases or of both.

30 What I claim is:

1. A method of making semipyrophoric iron from iron oxalate by thermal decomposition, which method consists in heating iron oxalate in the presence of indifferent gases maintaining the condition of reaction with respect to the duration of treatment within limits, above which pyrophoric and below which normal iron is obtained by the same treatment.

2. Semipyrophoric iron being a black powder 40 and whose ignition-point in contact with air is at about 180° C. produced by the method of claim 1.

ALFRED SCHMID.